

## 1

2,975,070

## VITREOUS ENAMEL

Burton C. Bricker, Wilmington, Del., and Lewis C. Hoffman, Scotch Plains, N.J., assignors to E. I. du Pont de Nemours and Company, Wilmington, Del., a corporation of Delaware

No Drawing. Filed Dec. 11, 1958, Ser. No. 779,525

1 Claim. (Cl. 106—49)

This invention relates to improved vitreous enamel coatings for aluminum and aluminum-rich alloys, i.e. alloys containing at least 80% of aluminum.

The first successful vitreous enamels for the enameling of aluminum and aluminum-rich alloys were developed by A. J. Deyrup and are fully disclosed in his U.S. Patent No. 2,467,114. Since this development, the vitreous enameling of aluminum has been practiced on a large scale, particularly for the use of such enamelled aluminum on the exterior of buildings.

Despite the success of aluminum enamels, continued difficulties have arisen in the consistent and uniform formation of hard, glossy, vitreous enamels of good adherence and resistance to the weathering influences under atmospheric conditions in all climates.

It is an object of this invention to produce an improved vitreous enamel coating for aluminum and aluminum-rich alloys.

It is another object to produce a vitreous enamel coating for aluminum and aluminum-rich alloys that will have an improved color stability.

It is a further object to produce a vitreous enamel coating for aluminum and aluminum-rich alloys that will have an improved weather resistance.

It is a still further object to produce a vitreous enamel coating for aluminum and aluminum-rich alloys that will have an improved opaqueness with a given content of opacifying agent.

Other objects of the invention will appear hereinafter.

It has now been found that a new and improved series of aluminum enamels can be prepared which, in comparison to previously known aluminum enamels, have a greatly reduced tendency to form the yellow devitrification product comprised of lead titanate, have a reduced tendency to dissolve opacifying agents, have up to 50% greater weathering or chemical resistance, are easily applied to aluminum without extensive pretreatment, do not objectionably corrode aluminum during application and firing, and have otherwise the desirable gloss and other properties of previously known aluminum enamels, for example, the enamels described and claimed in Deyrup, U.S. Patent No. 2,467,114.

In order to obtain the requisite chemical resistance it is desirable that the enamel composition contain at least about 19 mol percent of titanium dioxide. The presence of more than about 8% lead oxide in a vitreous composition containing more than about 19% titanium dioxide is very undesirable since the resulting frit may contain a considerable amount of lead titanate, which is subject to highly objectionable yellow devitrification upon slight over-firing. In reducing the lead oxide con-

## 2

tent of such a vitreous composition, it is necessary to increase the alkali metal oxide content to maintain a maturing temperature of below 1000° F. But, upon increasing the alkali metal oxide content beyond a limit, 5 the frit becomes too corrosive to the aluminum or aluminum alloy during coating and firing operations. Again, the presence of slightly too much K<sub>2</sub>O will produce a frit that is insufficiently acid or weather resistant. Too much Li<sub>2</sub>O causes the frit to dissolve too great a quantity 10 of opacifying agents, for example, TiO<sub>2</sub> or SnO<sub>2</sub>. As a consequence, it is exceedingly difficult to formulate a satisfactory enamel for purposes of enameling aluminum or aluminum-rich alloys. In the enamel of this invention a slight quantity of Sb<sub>2</sub>O<sub>3</sub> is useful to mitigate to 15 some extent the corrosive effects of alkali metal oxides, and BaO contributes thereto to maintain a low melting range and impart a corrosion resistance to the final enamels.

The new and improved vitreous enamels of this invention have a firing or maturing temperature between 920° F. and 1000° F. and contain the following constituents within the following ranges and proportions:

|                                                  | Mole percent |
|--------------------------------------------------|--------------|
| Lead oxide (PbO)                                 | 2-7          |
| Silicon oxide (SiO <sub>2</sub> )                | 33-37        |
| Titanium oxide (TiO <sub>2</sub> )               | 19-25        |
| Sodium oxide (Na <sub>2</sub> O)                 | 21-30        |
| Lithium oxide (Li <sub>2</sub> O)                | 0-6          |
| Potassium oxide (K <sub>2</sub> O)               | 0-10         |
| Antimony oxide (Sb <sub>2</sub> O <sub>3</sub> ) | 0-1          |
| Barium oxide (BaO)                               | 0-6          |
| Boron oxide (B <sub>2</sub> O <sub>3</sub> )     | 0-1          |
| Cadmium oxide (CdO)                              | 0-2          |

35 The total alkali metal oxide content (Li<sub>2</sub>O+Na<sub>2</sub>O+K<sub>2</sub>O) of the enamel composition must be between 33 and 37 mole percent, and the ratio of the silica content plus twice the titanium oxide content of the composition, in mole percent, to the alkali metal oxide content plus the lead oxide content, in mole percent, must be between 1.8 and 2.4, i.e.

$$\frac{\text{SiO}_2 + 2\text{TiO}_2}{\text{Li}_2\text{O} + \text{Na}_2\text{O} + \text{K}_2\text{O}} = 1.8 \text{ and } 2.4$$

45 Small percentages of other constituents than those above mentioned may be contained in the vitreous enamels of this invention. For example, such enamels may contain up to about 2% of Al<sub>2</sub>O<sub>3</sub>, 4% of SrO or CaO, 1% of CoO, 0.1% of MnO, 0.1% of NiO, 3% of ZnO or 4% of ZrO<sub>2</sub>; however at least 90% of content 50 of these enamels must consist of the above-named ingredients within the ranges stated.

The enamel constituents are expressed in mole percent as defining the invention more accurately than could 55 be done by weight percentages, however, for ready comparison with compositions expressed in weight percentages, the examples will be set forth in both weight and mole percentages.

60 The following three (3) tables disclose ten specific examples of compositions prepared in accordance with the invention. Table I discloses the compositions in mole percent and includes the aforesaid mole percent ratios, Table II in weight percent, and Table III in weight percent of the batch ingredients from which the vitreous 65 enamel frit is prepared.

TABLE I  
*Mole percent of melted compositions*

| Example No.                         | 1    | 2    | 3    | 4    | 5    | 6    | 7    | 8    | 9    | 10   |
|-------------------------------------|------|------|------|------|------|------|------|------|------|------|
| PbO                                 | 6.2  | 5.3  | 5.4  | 5.0  | 5.1  | 3.0  | 2.6  | 2.1  | 2.1  | 2.0  |
| SiO <sub>2</sub>                    | 36.3 | 34.6 | 34.5 | 35.5 | 34.9 | 35.3 | 34.1 | 34.4 | 34.4 | 33.3 |
| TiO <sub>2</sub>                    | 19.5 | 23.3 | 23.0 | 23.1 | 24.5 | 23.9 | 24.9 | 24.1 | 24.1 | 23.4 |
| Na <sub>2</sub> O                   | 23.4 | 26.8 | 26.7 | 26.5 | 24.3 | 23.7 | 23.7 | 23.9 | 20.9 | 29.8 |
| Li <sub>2</sub> O                   | 5.6  | 4.4  | 4.4  | 4.3  | 4.4  | 4.3  | 4.3  | 4.3  | 4.3  | 4.2  |
| K <sub>2</sub> O                    | 4.8  | 3.2  | 3.2  | 3.2  | 5.1  | 5.0  | 5.0  | 5.0  | 9.5  | 2.9  |
| Sb <sub>2</sub> O <sub>3</sub>      | 0.6  | 0.5  | 0.5  | 0.5  | 0.5  | 0.5  | 0.5  | 0.5  | 0.5  | 0.4  |
| BaO <sub>1</sub>                    | 0.1  |      |      |      |      |      |      | 0.2  | 0.2  | 0.2  |
| BaO <sub>2</sub>                    |      | 3.5  | 1.9  | 0.5  | 1.9  | 1.2  | 4.3  | 4.9  | 5.5  | 4.0  |
| CdO                                 |      |      | 1.8  |      |      |      |      |      |      |      |
| Mole Percent Ratio:                 |      |      |      |      |      |      |      |      |      |      |
| SiO <sub>2</sub> +2TiO <sub>2</sub> | 1.88 | 2.05 | 2.03 | 2.09 | 2.16 | 2.31 | 2.36 | 2.34 | 2.24 | 2.06 |
| R <sub>2</sub> O+PbO                |      |      |      |      |      |      |      |      |      |      |

TABLE II  
*Weight percent of melted compositions*

| Example No.                    | 1    | 2    | 3    | 4    | 5    | 6    | 7    | 8    | 9    | 10   |
|--------------------------------|------|------|------|------|------|------|------|------|------|------|
| PbO                            | 17.3 | 15.7 | 15.7 | 14.7 | 14.7 | 8.7  | 7.7  | 6.0  | 6.0  | 6.0  |
| SiO <sub>2</sub>               | 27.3 | 27.0 | 27.0 | 28.0 | 27.0 | 28.0 | 27.0 | 27.0 | 27.0 | 27.0 |
| TiO <sub>2</sub>               | 19.5 | 24.3 | 24.3 | 24.3 | 25.3 | 25.3 | 26.3 | 25.3 | 25.3 | 25.3 |
| Na <sub>2</sub> O              | 18.2 | 21.7 | 21.7 | 21.7 | 19.5 | 19.5 | 19.5 | 19.5 | 17.0 | 25.0 |
| Li <sub>2</sub> O              | 2.1  | 1.7  | 1.7  | 1.7  | 1.7  | 1.7  | 1.7  | 1.7  | 1.7  | 1.7  |
| K <sub>2</sub> O               | 5.7  | 4.0  | 4.0  | 4.0  | 6.2  | 6.2  | 6.2  | 6.2  | 11.7 | 3.7  |
| Sb <sub>2</sub> O <sub>3</sub> | 2.2  | 1.7  | 1.7  | 1.7  | 1.7  | 1.7  | 1.7  | 1.7  | 1.7  | 1.7  |
| B <sub>2</sub> O <sub>3</sub>  | 0.9  |      |      |      |      |      |      | 1.5  | 1.5  | 1.5  |
| BaO                            | 6.8  | 3.9  | 0.9  | 3.9  | 3.9  | 9.0  | 9.0  | 11.1 | 8.1  | 8.1  |
| CdO                            |      |      | 3.0  |      |      |      |      |      |      |      |

TABLE III  
*Batches in weight percent*

| Example No.                               | 1    | 2    | 3    | 4    | 5    | 6    | 7    | 8    | 9    | 10   |
|-------------------------------------------|------|------|------|------|------|------|------|------|------|------|
| PbO, Litharge                             | 14.3 | 13.0 | 13.1 | 12.2 | 12.2 | 7.1  | 6.3  | 4.8  | 4.7  | 4.8  |
| SiO <sub>2</sub> , Potters Flint          | 22.5 | 22.3 | 22.5 | 23.2 | 22.4 | 23.0 | 22.1 | 21.8 | 22.1 | 21.5 |
| TiO <sub>2</sub>                          | 16.1 | 20.1 | 20.2 | 20.1 | 21.0 | 20.8 | 21.5 | 20.4 | 19.8 | 20.1 |
| Na <sub>2</sub> CO <sub>3</sub>           | 25.5 | 30.7 | 30.9 | 30.7 | 27.7 | 27.3 | 27.3 | 26.9 | 24.7 | 34.0 |
| Li <sub>2</sub> CO <sub>3</sub>           | 4.1  | 3.4  | 3.4  | 3.4  | 3.4  | 3.4  | 3.4  | 3.3  | 3.2  | 3.3  |
| K <sub>2</sub> CO <sub>3</sub> , Calcined | 7.1  | 5.0  | 5.0  | 5.0  | 7.7  | 7.6  | 7.6  | 7.5  | 13.8 | 4.5  |
| Sb <sub>2</sub> O <sub>3</sub>            | 1.8  | 1.4  | 1.4  | 1.4  | 1.4  | 1.4  | 1.4  | 1.3  | 1.4  |      |
| H <sub>3</sub> BO <sub>3</sub>            | 1.3  |      |      |      |      |      |      | 2.2  | 2.1  | 2.2  |
| BaCO <sub>3</sub>                         | 7.3  | 4.1  | 1.0  | 4.0  | 4.2  | 9.6  | 10.4 | 11.7 | 8.3  | 8.2  |
| CdO                                       |      |      | 2.5  |      |      |      |      |      |      |      |

In preparing these frits, the batch is weighed, mixed, heated in a crucible until the mix is completely melted to a homogeneous glass. Crucible temperatures may vary within wide limits, but 900° C. to 1200° C. is a particularly suitable range. The molten glass is fritted by running into water which shatters it into small pieces forming the frit. The frit is advantageously freed of water by low-temperature drying, for example, at a temperature less than 50° C.

The frit is then placed, for grinding, in a ball mill or other mill, with water or other suitable liquid, or in some cases it may be dry-ground. Dry grinding may be preferred if the frit is to be stored for long periods because it obviates any attack of water on the comminuted frit and eliminates the operations of filtering and drying. If the frit is to be used directly in enamel, it is advantageously ground in water which serves as suspending medium for application to the metal articles. During the grinding, it is convenient to include with the frit white pigments (opacifying agents) such as titanium dioxide, or coloring pigments such as cobalt aluminate blue, in amounts up to 10% by weight of the total enamel compositions. These are, of course, omitted if a clear, colorless, vitreous coating is desired. It is advantageous also to include suitable dispersing and bonding agents as additions to the frit in the grinding mill. If the enamel is subject to tearing when applied and fired, anti-tearing agents, such as the alkali metal silicates and alkali metal

metaborate as described in U.S. Patent 2,653,877 should be added.

The dispersion or suspension of the powdered enamel in a suitable vehicle may be applied to the aluminum by the well-known procedures of spraying, dipping, stencilling, brushing, etc. As an example of a convenient vehicle for use in the spray application, one composed of methyl cellulose 0.75%, sodium chloride 1%, octyl alcohol 0.05%, and water 98.2% (all parts by weight) may be used; or commercial water glass (sodium silicate solution) 0.4%, sodium fluosilicate 0.4%, and water 99.2%. A suitable vehicle for applying the vitreous enamel by the squeegee-stencil application procedure is one composed of ethyl cellulose (25 c.p.s. viscosity grade) 4%, soya lecithin 0.25%, and terpineol 95.75%. When using aqueous vehicles for application, it is frequently desirable to include in the vehicle corrosion inhibitors to prevent the possible corrosion of the metal article by the enamel suspension, since such corrosion evolves hydrogen which may mechanically break up the enamel film before firing. Sodium silicate and fluosilicate may be used for this purpose, as in the vehicle cited above; or a small amount of soluble chromate such as 0.1% by weight of potassium chromate may be incorporated in the aqueous vehicle.

It is desirable to apply the enamel to the surface of the aluminum in any manner which will obtain a uniform and smooth coating before firing. The thickness of the coat may be varied within wide limits according to the type of

effect desired, although 15 to 30 grams (based on dry weight of enamel) per square foot per coat is generally preferred, several coats with separate firings being applied if desired. It is not generally necessary to apply any preliminary treatment to the surface of the aluminum or alloy other than removal of grease or excessive amounts of corrosion products except as described below. Usually these enamels may be applied to any aluminum or aluminum alloy surfaces without preliminary cleaning, provided the surface to be enameled is not contaminated. Cast metal articles to be enameled should be made with proper care to ensure dense castings free of undue porosity. In general, articles for enameling should be designed in accordance with the well-known principles obtained in other metal-enameling arts, particularly to avoid excessively sharp edges and corners in design. If such sharp edges, corners or burrs are present, they should be lightly rounded off by filing, grinding or other suitable means.

After application of the enamel to the metal, the composition is fired in a suitable furnace in order to fuse the powdered enamel to a continuous glassy coating. The firing conditions are not critical, except that the article must be brought to a temperature high enough to melt the enamel but not high enough to injure the metal article. The temperature necessary depends to some extent on the particular aluminum alloy being coated and on the particular enamel composition. However, it is not necessary to employ a temperature above 1000° F. and in some cases the enamel may be satisfactorily melted as low as 920° F. It is merely necessary to keep the article at the selected temperature for a few minutes to permit the enamel to fuse completely to a uniform, adherent, vitreous layer. Several coats may be applied, if desired. The firing, of course, should be effected in a furnace free of sulphate or chloride, or other objectionable fumes, which might impair the desired gloss. In some cases, the enameling may be advantageously combined with the heat treating of heat-treatable alloys. Long heat-treating periods, even of several hours' duration, generally do not adversely affect these enamels. When thin sheet stock is enameled, particularly of soft metals in this group such as pure aluminum sheet, it may be found to warp on cooling because of the differential contraction of metal and enamel during cooling. This may be obviated by enameling both sides of the sheet. Or, if desired, we find that, surprisingly, such warped sheet may be mechanically bent back to its original shape without any adverse effect on the enamel whatever. Or, if desired, warping difficulties may be minimized by use of the stronger alloys in fabricating articles for enameling.

Preferably, the aluminum or aluminum-rich alloy, prior to application of the enamels of this invention, is pretreated by the chromate treatment of Deyrup et al. as disclosed in U.S. Patent 2,544,139. Contrary to the method disclosed in that patent, the chromate-treated aluminum or aluminum alloy surfaces do not, in the case of some alloys, have to be pre-fired. Samples of an aluminum alloy sheet stock composed of aluminum alloy (containing by weight 0.25% copper, 0.6% silicon, 1% magnesium, and 0.25% chromium) is dipped into a bath consisting of

## Parts by weight

|                    |    |
|--------------------|----|
| Sodium hydroxide   | 4  |
| Potassium chromate | 20 |
| Water              | 76 |

and having a temperature of 50° C. After 5 minutes, the samples are withdrawn, rinsed with water, and dried at room temperature.

Each of these samples was coated with one of the specific examples of vitreous enamel disclosed in the above tables. Before coating, each enamel was provided with a mill addition consisting of 10% by weight of TiO<sub>2</sub> pigment and 7% by weight of a mixture of an anti-tearing agent consisting of

|                                                                                                          | Parts by weight |
|----------------------------------------------------------------------------------------------------------|-----------------|
| 10 Sodium hydroxide                                                                                      | 4.7             |
| Borax                                                                                                    | 22.2            |
| 15 Water glass solution, containing, by weight, 63% water and 37% Na <sub>2</sub> O·3.4 SiO <sub>2</sub> | 47.0            |
| 15 Water                                                                                                 | 26.1            |
|                                                                                                          | 100.0           |

The coated samples were fired for 10 minutes at a temperature of 960° F. and had the following properties

|                                                                                                                        |       |
|------------------------------------------------------------------------------------------------------------------------|-------|
| 20 Gloss: gloss/mil measured with a photovolt gloss-meter relative to a black glass standard angle of incidence 45°    | 75-80 |
| 25 Opacity: Reflectance percent measured with a photovolt reflectometer, green incident light relative to MgO standard | 80-83 |
| Corrosion resistance: Rating P.E.I. test, exposure to 10% citric acid for 15 minutes                                   | AA    |

30 All percentages referred to throughout the specification and claims, unless otherwise specifically stated, refer to mole percentages.

35 Since it is obvious that many changes and modifications can be made in the above-described details without departing from the nature and spirit of the invention, it is to be understood that this invention is not to be limited to said details except as set forth in the appended claim.

We claim:

40 A vitreous enamel frit, suitable for use as a protective coating on the surface of aluminum and aluminum-rich alloys, having a firing and maturing temperature below 1000° F., said frit consisting of the following, in mole percentages:

|                                | Percent |
|--------------------------------|---------|
| 45 PbO                         | 6.2     |
| SiO <sub>2</sub>               | 36.3    |
| TiO <sub>2</sub>               | 19.5    |
| Na <sub>2</sub> O              | 23.4    |
| Li <sub>2</sub> O              | 5.6     |
| 50 K <sub>2</sub> O            | 4.8     |
| Sb <sub>2</sub> O <sub>3</sub> | 0.6     |
| B <sub>2</sub> O <sub>3</sub>  | 0.1     |
| BaO                            | 3.5     |

55 all of said oxides being melted into said enamel composition.

## References Cited in the file of this patent

## UNITED STATES PATENTS

|                             |               |
|-----------------------------|---------------|
| 60 2,492,523 Coffeen et al. | Dec. 27, 1949 |
| 2,642,364 Beatty et al.     | June 16, 1953 |
| 2,909,438 Kautz             | Oct. 20, 1959 |

## FOREIGN PATENTS

|                          |               |
|--------------------------|---------------|
| 65 665,903 Great Britain | Jan. 30, 1952 |
|--------------------------|---------------|